

March 17, 1964

G. S. FOERSTER ET AL

3,125,444

MAGNESIUM BASE CASTING ALLOY

Filed April 3, 1963



INVENTORS

George S. Foerster  
Francis L. Burkett

BY

Griswold & Burdick  
ATTORNEYS

# United States Patent Office

3,125,444

Patented Mar. 17, 1964

1

3,125,444

## MAGNESIUM BASE CASTING ALLOY

George S. Foerster, Midland, and Francis L. Burkett, Breckenridge, Mich., assignors to The Dow Chemical Company, Midland, Mich., a corporation of Delaware

Filed Apr. 3, 1963, Ser. No. 279,246

6 Claims. (Cl. 75—168)

This invention relates to alloys of magnesium and particularly concerns a magnesium base alloy having particular utility as a casting alloy.

The object of the present invention is to provide a magnesium base alloy having improved castability and mechanical properties thus having particular utility as a casting alloy.

In general, the above and other objects and advantages have been found obtainable by adding to molten magnesium both aluminum and copper, each within a particular concentration range.

Accordingly, the alloy of the present invention comprises broadly an amount of aluminum by weight of from 5 to about 20 percent and an amount of copper by weight of from 4 to about 10 percent, the balance being magnesium. Specifically, however, the composition of the present alloy is graphically illustrated in the accompanying drawing, and thus conveniently determined therefrom. In the drawing there is shown on a conventional triangular coordinate graph the percent aluminum, percent copper and percent magnesium in the alloy. The alloy composition thus represented lies in a broad composition area and includes an area of preferred proportions, said areas being further defined below.

The amounts of aluminum and copper, the balance by difference being magnesium, which have been found satisfactory in the alloy of the present invention are shown graphically, as mentioned above, in the single figure of the drawing, the parallelogram ABCD thereof, bounded by lines AB, BC, CD and DA, referring to the broad composition range within which the aforesaid improved properties of the present alloy are obtained. The preferable composition range of the present alloy is also shown in said drawing as area DEFG, within the above parallelogram ABCD, bounded by lines DE, EF, FG and GD, said preferable composition area corresponding arithmetically in general to an amount of from about 5 to about 16 weight percent aluminum, and an amount of from about 5 to about 10 weight percent copper, the balance being magnesium.

In addition, small amounts of other alloying constituents conventionally employed may be used in the alloy provided it does not significantly impair the improved castability of the alloy obtained under the present invention.

The term magnesium, as referred to herein, means the pure metal and alloys thereof having less than about 1.0

2

In preparing the alloy of the present invention, magnesium is melted under a suitable halide flux cover using conventional melting and alloying techniques as practiced in the magnesium art, and the copper and aluminum added thereto as small ingots or chunks at a temperature sufficient to dissolve said additions, such as, for example, a temperature of from 1250 to about 1350° F. The alloy so prepared may be cast into ingots suitable for remelting and casting or cast directly after preparation into desired cast articles. In casting, the so-prepared melt is preferably cast in a heated mold having the desired cavity configuration, the mold being heated to a temperature of from about 300 to about 700° F. or more, such that premature solidification during pouring in the smaller and irregular channels, if any, in the mold cavity will not occur prior to completion of pouring and subsequent withdrawal of the heat source from the mold. After the mold is filled and the heating means withdrawn therefrom, the metal in the mold is allowed to cool sufficiently to solidify. The solidified cast article is then removed from the mold. In addition, if desired, the so-cast article may be subsequently solution heat treated and aged to enhance strength.

The alloy of the present invention may be cast into sand or permanent molds, or employed in operations using a cold-mold die casting apparatus as commonly used in the die casting art.

The following examples serve to further illustrate the present invention.

Various magnesium base alloys containing aluminum and copper were prepared according to the present invention, each having a composition as indicated in Table I, by melting commercial grade magnesium at a temperature of about 1300° F. under a suitable halide flux cover and adding thereto small chunks of the said aluminum and copper. A suitable halide flux cover, for example, is one comprising about 34% KCl, about 31% MgCl<sub>2</sub>, about 12% CaF<sub>2</sub>, about 13% MgO, and about 10% BaCl<sub>2</sub>. A permanent mold having the cavity configuration of a 1/4 inch diameter round test bar was heated to a temperature of about 540° F. and the prepared alloy cast therein. These bars were then tested for percent elongation (percent E) (using a 2 inch gauge section), tensile strength (TS), and tensile yield strength (TYS) (at a 0.2% offset) in the as-cast condition, after solution heat treatment, and after solution heat treatment with subsequent aging, at the temperatures and times as indicated in Table I, which in addition sets forth the results of these tests.

It should be understood that other heat treatments and aging conditions than those indicated in Table I can be employed with respect to the alloy of the present invention in order to obtain, for example, greater age hardening and higher strength.

Table I

| Example  | Composition <sup>1</sup> |            | As Cast   |              |    | After Solution Heat Treating for 16 Hrs. at 750° F. |              |    | After Solution Heat Treating and Aging 24 Hrs. at 350° F. |              |    |
|----------|--------------------------|------------|-----------|--------------|----|-----------------------------------------------------|--------------|----|-----------------------------------------------------------|--------------|----|
|          | Percent Al               | Percent Cu | Percent E | 1,000 p.s.i. |    | Percent E                                           | 1,000 p.s.i. |    | Percent E                                                 | 1,000 p.s.i. |    |
|          |                          |            |           | TYs          | TS |                                                     | TYs          | TS |                                                           | TYs          | TS |
| (1)----- | 9.2                      | 5.8        | 2.0       | 16           | 27 | 0.8                                                 | 17           | 29 | 2.0                                                       | 16           | 26 |
| (2)----- | 6.3                      | 8.7        | 1.0       | 15           | 24 | 1.0                                                 | 15           | 21 | 0.5                                                       | 15           | 22 |
| (3)----- | 15.0                     | 6.0        | 0.5       | 24           | 26 | 0.5                                                 | 20           | 28 | 0.5                                                       | 27           | 31 |
| (4)----- | 15.0                     | 9.6        | 0.5       | 25           | 28 | 0.5                                                 | 22           | 26 | 0.5                                                       | 24           | 33 |

<sup>1</sup> Balance, magnesium.

percent of other alloying constituents therein either as additions or as unavoidable impurities.

Among the advantages of the alloy are that it has the light weight characteristic of magnesium, the molten alloy

flows easily into and completely fills casting molds of intricate shape producing castings having a high strength to weight ratio, and is composed of readily available metals.

We claim:

1. A magnesium base alloy consisting essentially of aluminum and copper and magnesium, said alloy having a composition by weight within the composition range represented by the area ABCD of the graph in the appended drawing bounded by lines AB, BC, CD, and DA.

2. A magnesium base alloy consisting essentially of aluminum and copper and magnesium, in proportions represented by the area DEFG of the graph in the appended drawing and bounded by lines DE, EF, FG and GD.

3. A magnesium base alloy consisting essentially of about 9.2 weight percent aluminum, and about 5.8 weight percent copper, the balance being magnesium.

4. A magnesium base alloy consisting essentially of

about 6.3 weight percent aluminum, and about 8.7 weight percent copper, the balance being magnesium.

5. A magnesium base alloy consisting essentially of about 15.0 weight percent aluminum and about 6.0 weight percent copper, the balance being magnesium.

6. A magnesium base alloy consisting essentially of about 15.0 weight percent aluminum and about 9.6 weight percent copper, the balance being magnesium.

10

**References Cited in the file of this patent**

**UNITED STATES PATENTS**

|           |         |       |                |
|-----------|---------|-------|----------------|
| 1,729,339 | Gann    | ----- | Sept. 24, 1929 |
| 1,793,023 | Schmidt | ----- | Feb. 17, 1931  |
| 2,314,024 | Topping | ----- | Mar. 16, 1943  |

15

**FOREIGN PATENTS**

|         |               |       |               |
|---------|---------------|-------|---------------|
| 293,359 | Great Britain | ----- | Jan. 31, 1929 |
|---------|---------------|-------|---------------|